# EUROPEAN PATENT SPECIFICATION

(11) **EP 0 734 429 B1**
(45) Date of publication and mention of the grant of the patent: **18.04.2001**
(21) Application number: 95904872.9
(22) Date of filing: 13.12.1994
(51) Int. Cl.: C10L 1/02

(54) **USE OF TERTIARY-HEXYL METHYL ETHER AS A MOTOR GASOLINE ADDITIVE**
VERWENDUNG VON T-HEXYL METHYLÄTHER ALS ADDITIV FÜR MOTORBENZIN
UTILISATION D'ETHER D'HEXYLE METHYLE TERTIAIRE COMME ADDITIF POUR ESSENCE MOTEUR

(30) Priority: 15.12.1993 US 167390
(43) Date of publication of application: 02.10.1996
(73) Proprietor: EXXON CHEMICAL PATENTS INC., Baytown, TX 77520-2149 (US)
(72) Inventor: HENDRIKSEN, Dan, Eldon, Kingwood, TX 77345 (US)
(74) Representative: White, Nicholas John, Dr.
(86) International application number: US9414234
(87) International publication number: WO9516763

(56) References cited:
- EP-A- 0 036 260
- EP-A- 0 254 496
- WO-A-89/11463
- US-A- 4 519 809

## Description

This invention relates to the use of one isomer of tertiary-hexyl methyl ether, which is 2-methoxy-2,3-dimethylbutane, as an octane booster in motor gasoline.

Generally, any component that has a research octane number over 105 and a motor octane number over 95 is considered to be an octane booster for use in motor gasoline. It is well known in the art that ethers made from C₄ and C₅ olefins are excellent octane boosters. Methyl tertiary-butyl ether (MTBE) made from isobutene, a C₄ olefin, has a research octane number (RON) of 118 and a motor octane number (MON) of 100; and tertiary-amyl methyl ether (TAME) produced from C₅ olefins has a RON of 111 and a MON of 98 according to Unzelman, Oil & Gas Journal, Volume 44, April 15, 1991.

It is also well known that these ethers have a higher octane booster number than their counterpart olefins. "Physical Constants of Hydrocarbon and Non-Hydrocarbon Compounds" ASTM data series publication DS 4B, 1991 states that the octane numbers for one of the parent olefins of TAME, 2-methyl-2-butene, is 97 for the RON and 82 for the MON. Etherification of this C₅ olefin increases the octane numbers to 111 for the RON and 98 for the MON. While the art teaches that ethers produced from C₄ and C₅ olefins are excellent octane boosters, it teaches away from the use of ethers produced from C₆ and heavier olefins.

For example, in Pescarollo et al.'s article, "Etherify light gasolines", Hydrocarbon Processing, February 1993, pp 53-60, he states that " ... ethers derived from C₆ and heavier olefins do not significantly enhance octane over the parent olefins".

Also, US-A-4,193,770, and its equivalent, DE-A-2,854,250 (1979) teaches that the octane numbers of the C₆ ethers are no higher than those of the parent olefins mixed with the same amount of methanol. The blending octane numbers for tertiary-hexyl methyl ether which is produced from a C₆ olefin are reported as being 100 for the RON and 90 for the MON, but no mention is made of any specific isomers, including 2-methoxy-2,3-dimethylbutane (MDMB). Hence, there is no recognition or teaching that MDMB is effective as an octane booster. The reported numbers serve to teach away from investigating the performance of ether produced from C₆ or C₇ olefins.

This reference teaches the importance of etherifying C₄ and C₅ olefins separately from each other because of the different reaction kinetics. Also stressed is the importance of keeping each of these fractions separate from the C₆ olefin fraction, which forms tertiary hexyl methyl ether, because there is no improvement in octane rating as compared to the ethers from the C₄ and C₅ olefins. The reference goes as far as saying that any reported increases in octane rating for ethers from C₆ and C₇ olefins, are "illusory". See column 3, lines 5 to 13 and 26 to 37.

This reference sets up a major prejudice against using C₆ ethers as motor gasoline octane boosters. And there is absolutely no mention of MDMB.

MICROLOG-88-03391 from Energy Res. Abstr., 13(22), Abstr. No. 5031, 1988, also teaches against the use of ethers produced from C₆ olefins in that "predictions for C₆ ethers were not carried out because there was virtually no improvement in octane number when compared with its precursors".

EP-A-0 036 260, discloses the use of ethers produced from a mixture of C₄ through C₇ olefins as components in a motor gasoline blend from a refinery catalytic cracker unit, with 7% being C₆ olefins, but reinforces the belief that the octane booster effect is due to the ethers produced from C₄ and C₅ olefins rather than those ethers produced from C₆ or C₇ olefins.

It would be desirable if ethers produced from C₆ olefins could be used as motor octane boosters. Current market predictions indicate that there will be a glut of propylene, which could be used to make C₆ olefins, in the market place within the next ten years. Currently, propylene is sent to the motor gasoline pool from refinery catalytic crackers, but the propylene does not boost the octane. It would be very profitable if one could determine a way to convert propylene into an octane booster.

### SUMMARY OF THE INVENTION

This invention relates to using an octane boosting amount of a tertiary hexyl methyl ether component comprising 2-methoxy-2,3-dimethyl butane (MDMB) which enables providing a blend comprising
(a) motor gasoline or motor gasoline feedstock; and
(b) an octane boosting amount of a tertiary hexyl methyl ether component comprising 2-methoxy-2,3-dimethyl butane (MDMB) in an amount of at least 10% by weight based on the total weight of tertiary hexyl methyl ether,
wherein composition (b) has a Research Octane Number (RON) and/or a Motor Octane Number (MON) greater than those of composition (a).

One embodiment includes providing a blend wherein the tertiary hexyl methyl ether component of composition (b) comprises in various amounts and ranges, including, greater than 10%, preferably from 20 to 100%, more preferably greater than 50%, even more preferably from 60% to 100%, and most preferably greater than 80% by weight of MDMB.

Another embodiment includes providing a blend wherein composition (b) contains greater than 50%, preferably from 60% to 100%, and more preferably greater than 80%, by weight of the tertiary hexyl methyl ether.

Yet another embodiment includes providing a method of increasing the octane number in motor gasoline comprising blending MDMB with the motor gasoline or with a motor gasoline feedstock to boost the octane number of the motor gasoline or motor gasoline feedstock which contains a sufficient amount of composition (b) to boost the octane number of component (a) by at least 1, preferably by at least 2, and more preferably by at least 3 units.

Still another embodiment includes the use of a tertiary hexyl methyl ether component comprising MDMB and having a blending RON greater than 100 and a blending MON greater than 90, as an octane booster for motor gasoline.

The tertiary hexyl methyl ether component comprising MDMB may be prepared by dimerizing propylenes and additional embodiments of the present invention include a blend wherein composition (b) is made by a process comprising:
(i) dimerizing propylene to form dimethylbutenes; and
(ii) etherifying the dimethyl butenes with methanol, to form the desired composition and/or a blend.

Additionally, another embodiment includes the further treatment wherein step (ii) comprises partial etherification and is followed by (iii) hydrogenation of unetherified dimethylbutenes to form a tertiary hexyl methyl ether composition comprising MDMB and dimethyl butanes.

### DETAILED DESCRIPTION OF THE INVENTION

Not all of the isomers of tertiary-hexyl methyl ether produced from C₆ olefins are suitable for use as octane boosters. The four isomers of tertiary-hexyl methyl ether (C₆ H₁₃-OCH₃) are as follows:
1) 2-Methoxy-2,3-dimethylbutane (MDMB)
2) 2-Methoxy-2-methylpentane (2MMP)
3) 3-Methoxy-3-methylpentane (3MMP)
4) 1-Methoxy-1-methylcyclopentane (MMCP)

1-Methoxy-1-methylcyclopentane (MMCP) is considered an isomer of tertiary-hexyl-methyl ether even though it has two fewer hydrogen atoms.

One isomer of tertiary-hexyl methyl ether has been found to be a very useful high octane booster for use in motor gasoline. That particular isomer is 2-methoxy-2,3-dimethylbutane (MDMB).

MDMB may be prepared from propylene and methanol by first dimerizing the propylene to dimethylbutenes (2,3-dimethyl)-(1 and/or 2)-butene), and then by etherifying the dimethylbutenes with methanol, as shown in the following reaction equations. Both 2,3-dimethyl-1-butene and 2,3-dimethyl-2-butene react with methanol to form the desired product ether.

Olefin dimerization and codimerization processes are known in the art. The propylene may be dimerized to dimethylbutenes (DMB) using a tungsten catalyst, such as that disclosed in U.S. Patent 5,059,739. The dimethylbutenes (DMB) may also be produced using nickel with specific organo-phosphine ligands.

In the event, the tungsten catalyst is used, the ratio of olefin to tungsten should be such that a catalytic amount of the tungsten complex is used. The reaction may be run in either a batch or a continuous manner. The reaction pressure is normally the pressure generated by the olefin at the reaction temperature, although the pressure may be increased with an inert gas. The reaction temperature may range, for example, from about 40 to 100°C, with 50 to 80°C being preferred. The reaction or residence time may be, for example, from 5 minutes to about 3 hours, with 0.5 to 2.0 hours being preferred. The preferred embodiment uses a catalyst which is prepared by taking a tungsten salt and an aniline to form a complex of the tungsten salt and aniline. Substantially all of the hydrogen chloride produced in this reaction is removed from the solution during the course of the reaction. After formation of the tungsten and aniline complex, an alkyl aluminum halide is added to the solution to form the active catalyst system of the invention. The preferred feedstock is refinery grade propylene, after sufficient removal of water and other catalyst poisons.

The etherification of the dimethylbutenes with methanol to prepare MDMB may take place in a manner similar to the preparation of methyl tertiary-butyl ether (MTBE) from isobutylene or the preparation of tertiary-amyl methyl ether (TAME) from isoamylenes. The reaction takes place over the acid form of an ion exchange resin.

The present invention involves the feeding of a mixture containing DMB and methanol into the feed zone of a reactor (i.e., a fixed-bed guard reactor), and contacting the resultant mixture of DMB and methanol with a fixed bed acidic cation exchange resin (e.g., Amberlyst® 15) in the reaction zone, thereby catalytically reacting the DMB with the methanol under conditions which favor forming the resultant 2-methoxy-2,3-dimethylbutane (MDMB).

Where the etherification step of the present invention is practiced in a catalytic distillation process, the catalytic material may be in any form which permits its incorporation into a distillation tower, such as a fixed bed, but may also be in a form which serves as a distillation packing, for example, rings, saddles, balls, irregular pieces, sheets, tubes, spirals, packed in bags, plated on grills or screens, and reticulated polymer foams.

Catalysts which have been found to be suitable for use in the etherification step of the present invention are resin catalysts such as cation exchange resin catalysts, acidic resin catalysts, macroreticular sulfonic acid cation exchange resin catalysts, and solid acid catalysts. Still others have used a zeolite as an etherification catalyst. Preferred catalysts for purposes of the present invention, however, are acid catalysts, such as acidic resin catalysts. A more preferred catalyst for purposes of the present invention is a macroreticular sulfonic acid cation exchange resin such as a sulfonated copolymer of polystyrene-divinyl-benzene. Such catalysts include Amberlyst ® 15 and 15C (marketed by Rohm and Haas), Lewatit SPC 118 and SPC 118 BG (marketed by Miles/Bayer), and Dowex M-31 and M-32 (marketed by the Dow Chemical Co.). A special version of this type of catalyst, i.e., Dowex DR-2040 (marketed by the Dow Chemical Co.), is used specifically for reactive distillation.

It has been found that equilibrium conversion to ether is only 50-60%, so it is expected that catalytic distillation will be advantageous in the etherification step. Catalytic distillation is commercially practiced in the production of MTBE and this process has been extensively explored with TAME. Therefore, there is every reason to expect that catalytic distillation would be advantageous when applied to the process for producing ethers from C₆ olefins.

When the ether is produced from a C₆ olefin which has been formed by dimerizing propylene, the composition of the resulting mixture of isomers may be as pure as 98 wt% MDMB, 2 wt% 2MMP, with negligible amounts of 3MMP and MMCP. When the C₆ olefin is produced in a refinery catalytic cracker, the isomer mixture is different, with more than 50% being 2MMP and approximately 7% being MDMB.

It is well known in the art that ethers are used as motor gasoline additives to enhance the quality of the motor gasoline due to environmental regulations, both existing and pending in the USA. By using an oxygenate rather than its counter part olefin in motor gasoline, less carbon monoxide pollution is produced upon combustion of the motor gasoline. Also, the rules regulating reformulated gasoline, which is a particular type of motor gasoline, require that a lower olefin content be present in the gasoline due to the fact that olefins contribute to ozone formation more than their counter part ethers. An additional advantage of using the ether rather than the olefin in motor gasoline is that the ether has a lower Reid vapor pressure, which reduces evaporative emissions which contribute to pollution.

The addition of the MDMB to the motor gasoline or motor gasoline feedstock to boost the octane may be accomplished in several ways. One method includes the preparation of a blend comprising the mixture of two compositions, (a) and (b), wherein composition (a) consists of the motor gasoline or motor gasoline feedstock which is blended with composition (b) which comprises an octane boosting amount of a tertiary hexyl methyl ether component comprising 2-methoxy-2,3-dimethyl butane (MDMB) in an amount of at least 10% by weight based on the total weight of tertiary hexyl methyl ether, wherein the composition (b) has a Research Octane Number (RON) and/or a Motor Octane Number (MON) greater than those of composition (a).

In addition to the tertiary hexyl methyl ethers and the MDMB, composition (b) may include other components. These additional components may be any other hydrocarbons typically found in motor gasoline or motor gasoline feedstocks, including, but not limited to, aromatics, olefins, and saturates.

These additional hydrocarbons may or may not be considered useful as octane boosters. In the case where the other hydrocarbons are useful as octane boosters, composition (b) may include either MTBE or TAME, or mixtures thereof.

Composition (b) may have a RON greater than 95, preferably greater than 100, and/or a MON greater than 85, preferably greater than 90.

Optionally composition (b) has a blending RON greater than 100, preferably greater than 105 and/or a blending MON greater than 90, preferably greater than 95.

The tertiary hexyl methyl ether component of composition (b) may comprise greater than 10%, preferably from 20 to 100%, by weight of MDMB. Optionally, this tertiary hexyl methyl ether component of composition (b) may comprise from 50 to 100%, preferably greater than 80%, by weight of MDMB.

The tertiary hexyl methyl ether component may have a RON greater than 100 and/or a MON greater than 90. Optionally, this tertiary hexyl methyl ether component may have a blending RON greater than 100 and/or a blending MON greater than 90.

The MDMB component of composition (b) may have a RON greater than 105 and/or a MON greater than 95. Optionally, the MDMB component may have a blending RON greater than 105 and/or a blending MON greater than 95.

The resulting blend may have a RON greater than 90, preferably greater than 93, and/or a MON greater than 80, preferably greater than 83.

A sufficient amount of composition (b) must be blended with composition (a) such that the octane number of component (a) is boosted by at least 1, preferably by at least 2, and more preferably by at least 3 units. The resulting blend may which comprise greater than 1%, preferably greater than 2%, and most preferably greater than 5 %, by volume of MDMB.

In addition to its use as an octane booster, MDMB has the added benefit of not significantly increasing the Reid vapor pressure (RVP) of the motor gasoline blend as is typical with other octane boosters, such as MTBE or TAME.

For example, MTBE has a blending RVP of 57.9 kPa (8.4 psi) and TAME has a blending RVP of 27.6 kPa (4.0 psi), both of which are higher than that of MDMB being 6.9 kPa (1 psi).

When the starting motor gasoline feedstock has a high RVP level, one could be limited on how much MTBE or TAME addition is possible to achieve the required octane requirements, while at the same time, not exceeding the RVP limit.

Therefore, an additional embodiment of the present invention includes the use of more than one octane booster to achieve the maximum octane boosting effect and without the corresponding undesirable increase in RVP.

For example, one could make a blend comprising the addition of MTBE and/or TAME up to the maximum RVP limit of the motor gasoline product as set by an environmental standard. Then, MDMP, either alone or in mixture with the tertiary hexyl methyl ether, could be blended into the motor gasoline to achieve on even higher octane number without incurring any increase in the RVP of the final blend of motor gasoline.

One embodiment of the invention includes a blend which contains a sufficient amount of composition (b) to boost the octane number of component (a) by at least 1, while at the same time increasing the Reid vapor pressure of component (a) by less than 13.8 kPa (2 psi), preferably by less than 6.9 kPa (1 psi), and more preferably by less than 3.4 kPa (0.5 psi).

The MDMB may be prepared using a process comprising (i) dimerizing propylene to form dimethylbutenes and (ii) etherifying the dimethyl butenes with methanol. Optionally, wherein step (ii) comprises partial etherification, the process may further comprise the additional step of (iii) hydrogenation of the unetherified dimethylbutenes to form a tertiary hexyl methyl ether composition comprising MDMB and dimethyl butanes.

Composition (b) may contain dimethylbutenes and may also contain less than 1% methanol and/or less than 5% olefins. Composition (b) may contain greater than 50%, preferably from 60% to 100%, and more preferably greater than 80%, by weight of the tertiary hexyl methyl ether.

By blending the prepared MDMB, with a motor gasoline or motor gasoline feedstock, the octane number of the blended gasoline may be increased by 1 or more units, preferably 2 or more units, and most preferably 3 or more units, over the original octane number of the motor gasoline or motor gasoline feedstock.

The foregoing invention will now be illustrated by, although not limited to, the following examples.

### EXAMPLES

### EXAMPLE I

### 2-MMP Comparative Example

This comparative example illustrates that not all ethers produced from C₆ olefins are useful as octane boosters.

An ion exchange resin in the acid form (Amberlyst R15, washed with methanol) was added to a 5000 mL round-bottom flask along with 1000 g of 2-methyl-1-pentene and 416 g methanol. The slurry of resin catalyst was stirred magnetically and refluxed at atmospheric pressure for 16 hours. In the refluxing process, the material boils at atmospheric pressure and condenses the vapors back into the boiling material. The resin catalyst was filtered from the product mixture, and then unconverted methanol and methyl pentenes were distilled away from the product ether (2MMP). The unconverted materials were placed back in the reaction flask with the resin catalyst and refluxed again for another 16 hours. This procedure of reaction followed by removal of product ether was repeated three times. This was desirable in order to achieve good conversion of the starting material since the etherification reaction is equilibrium limited. The product ether was distilled again (boiling point 112°C) to yield product purity of 99.4% by GC analysis.

The octane numbers and Reid vapor pressure results were measured using the standard test methods well known in the art. The Research Octane Number (RON) was 88.3 and the Motor Octane Number (MON) was approximately 90. The precise MON could not be measured as the fuel/air ratio was set at the highest setting available on the test engine. In the standard test procedure, the fuel/air ratio is continually increased until maximum knock is obtained. The Reid vapor pressure was 8.6 kPa (1.25 psi).

These results are consistent with the reported octane numbers for ethers of C₆ olefins, and support the industry view (for example, as expressed in US-A-4,193,770) that such ethers are not useful as octane boosters for motor gasoline.

### EXAMPLE II

### MDMB - the Invention

This example of the invention illustrates that one of the ethers produced from C₆ olefins, specifically MDMB, is useful as an octane booster.

2-Methoxy-2,3-dimethyl butane (MDMB) was prepared from 2,3-dimethyl-2-butene (2112 g) and methanol (879 g) in a similar manner as described for preparation of 2MMP in Example I. The product had a boiling point of 115°C and a product purity of 98.2% 2-methoxy-2,3-dimethylbutane with the balance being 2-methoxy-2-methyl pentane from 2-methylpentene impurity in the starting material. The Research Octane Number measured for this MDMB rich product was 108.1 and the Motor Octane Number was 96.8. The Reid vapor pressure was 7.3 kPa (1.06 psi).

### Analysis of Examples I and II

The octane numbers from Examples I and II along with those of C₄ and C₅ olefins are reproduced below in a table format for easy comparison.

| Parent Olefin | Ether | RON | MON |
|---|---|---|---|
| C₄ | MTBE | 118 | 100 |
| C₅ | TAME | 111 | 98 |
| C₆ | MDMB | 108.1 | 96.8 |
| | 2MMP | 88.3 | approximately 90 |

One can see that unexpectedly, and contrary to the prejudice arising from the prior art investigation of C₆ olefin ether, MDMB has RON and MON values which make it surprisingly good as an octane booster for motor gasoline.

### EXAMPLE III

In addition to the component RON, MON, and Reid vapor pressure (RVP) numbers being determined, a set of corresponding blending values for MDMB was also ascertained. As it is well known to one of ordinary skill in the art, the "blending" RON, MON, and RVP values vary based upon the base gasoline composition. Typically, the "Blending Values" (BV) are higher for RON and MON and are slightly lower for RVP.

Blends of approximately 14, 19, and 25% volume MDMB/volume gasoline, as synthesized in Example II, were prepared using two different gasolines, A and B, as described below.

| | Gasoline A | Gasoline B |
|---|---|---|
| RON | 93 | 97 |
| MON | 83 | 87 |
| RVP, kPa | 50.3 (7.3 psi) | 53.8 (7.8 psi) |

The resulting RON, MON, and Reid vapor pressure numbers were measured for each of the blends with the following results.

| Gasoline | MDMB Vol % | RON Blend | MON Blend | RVP Blend, kPa | RVP Blend, psi |
|---|---|---|---|---|---|
| A | 13.8 | 95.6 | 85.2 | 45.5 | 6.6 |
| A | 18.7 | 96.3 | 85.8 | 43.4 | 6.3 |
| A | 24.3 | 97.3 | 87.0 | 37.9 | 5.5 |
| Average A | ---- | 96.4 | 86.0 | 42.1 | 6.1 |
| B | 14.2 | 98.8 | 88.2 | 42.7 | 6.2 |
| B | 19.2 | 99.4 | 88.8 | 46.2 | 6.7 |
| B | 24.9 | 99.9 | 89.6 | 40.7 | 5.9 |
| Average B | ---- | 99.4 | 88.7 | 43.4 | 6.3 |

The values of the blend were then used in the following manner to calculate the properties of the finished blend. RVP is used as an example.${\text{RVP}}_{\text{blend}} \text{=} \frac{{\text{VOL}}_{\text{gasoline}}}{{\text{VOL}}_{\text{gasoline}} {\text{+ VOL}}_{\text{MDMB}}} {\text{* RVP}}_{\text{gasoline}} \text{+} \frac{{\text{VOL}}_{\text{MDMB}}}{{\text{VOL}}_{\text{gasoline}} {\text{+ VOL}}_{\text{MDMB}}} {\text{* BV RVP}}_{\text{MDMB}}$

Even though this equation is not 100% accurate for calculating octane numbers, as the RON and MON do not blend linearly, it can be used to predict octane within ±1 number for the narrow range of blends investigated.

This example illustrates that the blending values for the properties of MDMB for the RON and MON are somewhat higher with an average of 110 and 97 respectively, and the RVP is somewhat lower at 6.9 kPa (1 psi), which is typical, as compared to the component values for the RON, MON, and RVP of the MDMB component, which were 108, 97, and 7.3 kPa (1.06 psi) respectively. Also shown for reference are the typical blending values for 15% MTBE, 10% ethanol and 12% TAME.

| COMPONENT | RON BV | MON BV | RVP BV |
|---|---|---|---|
| MDMB with Gasoline A | 112 | 98 | 1 |
| MDMB with Gasoline B | 109 | 96 | 1 |
| MTBE | 117 | 98 | 8.4 |
| ETHANOL | 115 | 96 | 22 |
| TAME | 106 | 94 | 224 |

One can see that the blending RON and MON values of MDMB are comparable to those of MTBE, ethanol, and TAME, which makes MDMB attractive as an octane booster for motor gasoline. MDMB's low blending RVP value makes it especially attractive as an octane booster in comparison to MTBE, ethanol, and TAME, as it does not carry a high RVP debit as is typically associated with the other octane boosters.

## Claims

1. A blend comprising
(a) motor gasoline or motor gasoline feedstock; and
(b) an octane boosting amount of a tertiary hexyl methyl ether component comprising 2-methoxy-2,3-dimethyl butane (MDMB) in an amount of at least 10% by weight based on the total weight of tertiary hexyl methyl ether,
wherein the composition (b) has a Research Octane Number (RON) and/or a Motor Octane Number (MON) greater than those of composition (a).

2. A blend according to Claim 1, wherein the composition (b) has a RON greater than 95 and/or a MON greater than 85.

3. A blend according to any preceding claim, wherein the composition (b) has a RON greater than 105 and/or a MON greater than 95.

4. A blend according to any preceding claims, wherein the tertiary hexyl methyl ether component of composition (b) comprises greater than 10%.

5. A blend according to any preceding claims, wherein the tertiary hexyl methyl ether component of composition (b) comprises from 20 to 100%, by weight of MDMB.

6. A blend according to any of the preceding claims, wherein the tertiary hexyl methyl ether component of composition (b) comprises from 50 to 100%.

7. A blend according to any of the preceding claims, wherein the tertiary hexyl methyl ether component of composition (b) comprises greater than 80%, by weight of MDMB.

8. A blend according to any of the preceding claims, wherein the tertiary hexyl methyl ether component has a RON greater than 100 and/or a MON greater than 90.

9. A blend according to any of the preceding claims, wherein the tertiary hexyl methyl ether component has a blending RON greater than 100 and/or a blending MON greater than 90.

10. A blend according to any of the preceding claims, wherein the MDMB component has a RON greater than 105 and/or a MON greater than 95.

11. A blend according to any of the preceding claims, wherein the MDMB component has a blending RON greater than 105 and/or a blending MON greater than 95.

12. A blend according to any of the preceding claims, wherein the blend has a RON greater than 90 and/or a MON greater than 80.

13. A blend according to any of the preceding claims, wherein the blend has a RON greater than 93 and/or a MON greater than 83.

14. A blend according to any of the preceding claims, which contains a sufficient amount of composition (b) to boost the octane number of component (a) by at least 1, preferably by at least 2, and more preferably by at least 3 units.

15. A blend according to any of the preceding claims, which comprises greater than 1%, preferably greater than 2%, and most preferably greater than 5%, by volume of MDMB.

16. A blend according to any of the preceding claims, wherein composition (b) is made by a process comprising:
(i) dimerizing propylene to form dimethylbutenes; and
(ii) etherifying the dimethyl butenes with methanol,
to form the desired composition.

17. A blend according to Claim 16, wherein step (ii) comprises partial etherification and is followed by
(iii) hydrogenation of unetherified dimethylbutenes
to form a tertiary hexyl methyl ether composition comprising MDMB and dimethyl butanes.

18. A blend according to any preceding claim, wherein composition (b) also contains dimethylbutenes.

19. A blend according to any preceding claim, wherein composition (b) also contains less than 1% methanol.

20. A blend according to any preceding claim, wherein composition (b) also contains less than 5% olefins.

21. A blend according to any preceding claim, wherein composition (b) contains greater than 50%, preferably from 60% to 100%, and more preferably greater than 80%, by weight of the tertiary hexyl methyl ether.

22. A blend according to any of the preceding claims, which contains a sufficient amount of composition (b) to boost the octane number of component (a) by at least 1 unit, while at the same time increasing the Reid vapor pressure of component (a) by less than 13.8 kPa (2 psi), preferably by less than 6.9 kPa (1 psi), and more preferably by less than 3.4 kPa (0.5 psi).

23. The use of a tertiary hexyl methyl ether component comprising MDMB in an amount of at least 10% by weight based on the total weight of tertiary hexyl methyl ether component and having a blending RON greater than 100 and a blending MON greater than 90, as an octane booster for motor gasoline.

24. The use of a tertiary hexyl methyl ether component comprising MDMB in an amount of at least 10% by weight based on the total weight of tertiary hexyl methyl ether component, as an octane booster for motor gasoline wherein the blending RON and/or the blending MON of the tertiary hexyl methyl ether component is higher than the RON and/or MON of the untreated motor gasoline.

25. The use of a tertiary hexyl methyl ether component in accordance with Claim 23 or 24, wherein the Reid vapor pressure of the treated motor gasoline is higher by less than 13.8 kPa (2 psi), preferably by less than 6.9 kPa (1 psi), and more preferably by less than 3.4 kPa (0.5 psi).

## Patentansprüche

1. Gemisch, das
(a) Motorbenzin oder Motorbenzineinsatzmaterial, und
(b) eine die Oktanzahl steigernde Menge einer tert.-Hexylmethyletherkomponente umfasst, die 2-Methoxy-2,3-dimethylbutan (MDMB) in einer Menge von mindestens 10 Gew.%, bezogen auf das Gesamtgewicht von tert.-Hexylmethylether, umfasst,
wobei die Zusammensetzung (b) eine Research-Oktanzahl (RON) und/oder eine Motoroktanzahl (MON) größer als diejenigen der Zusammensetzung (a) aufweist.

2. Gemisch nach Anspruch 1, bei dem die Zusammensetzung (b) eine RON größer als 95 und/oder eine MON größer als 85 hat.

3. Gemisch nach einem der vorhergehenden Ansprüche, bei dem die Zusammensetzung (b) eine RON größer als 105 und/oder eine MON größer als 95 hat.

4. Gemisch nach einem der vorhergehenden Ansprüche, bei dem die tert.-Hexylmethyletherkomponente der Zusammensetzung (b) mehr als 10 % umfasst.

5. Gemisch nach einem der vorhergehenden Ansprüche, bei dem die tert.-Hexylmethyletherkomponente der Zusammensetzung (b) 20 bis 100 Gew.% MDBD umfasst.

6. Gemisch nach einem der vorhergehenden Ansprüche, bei dem die tert.-Hexylmethyletherkomponente der Zusammensetzung (b) 50 bis 100 % umfasst.

7. Gemisch nach einem der vorhergehenden Ansprüche, bei dem die tert.-Hexylmethyletherkomponente der Zusammensetzung (b) mehr als 80 Gew.% MDMB umfasst.

8. Gemisch nach einem der vorhergehenden Ansprüche, bei dem die tert.-Hexylmethyletherkomponente eine RON größer als 100 und/oder eine MON größer als 90 hat.

9. Gemisch nach einem der vorhergehenden Ansprüche, bei dem die tert.-Hexylmethyletherkomponente eine Misch-RON größer als 100 und/oder eine Misch-MON größer als 90 hat.

10. Gemisch nach einem der vorhergehenden Ansprüche, bei dem die MDMB-Komponente eine RON größer als 105 und/oder eine MON größer als 95 hat.

11. Gemisch nach einem der vorhergehenden Ansprüche, bei dem die MDMB-Komponente eine Misch-RON größer als 105 und/oder eine Misch-MON größer als 95 hat.

12. Gemisch nach einem der vorhergehenden Ansprüche, bei dem das Gemisch eine RON größer als 90 und/oder eine MON größer als 80 hat.

13. Gemisch nach einem der vorhergehenden Ansprüche, bei dem das Gemisch eine RON größer als 93 und/oder eine MON größer als 83 hat.

14. Gemisch nach einem der vorhergehenden Ansprüche, das eine ausreichende Menge Zusammensetzung (b) enthält, um die Oktanzahl von Komponente (a) um mindestens 1, vorzugsweise mindestens 2 und insbesondere mindestens 3 Einheiten zu steigern.

15. Gemisch nach einem der vorhergehenden Ansprüche, das mehr als 1 Vol.%, vorzugsweise mehr als 2 Vol.% und am meisten bevorzugt mehr als 5 Vol.% MDMB umfasst.

16. Gemisch nach einem der vorhergehenden Ansprüche, bei dem Zusammensetzung (b) nach einem Verfahren hergestellt ist, bei dem
(i) Propylen dimerisiert wird, um Dimethylbutene zu bilden, und
(ii) die Dimethylbutene mit Methanol verethert werden,
um die gewünschte Zusammensetzung zu bilden.

17. Gemisch nach Anspruch 16, bei dem Stufe (ii) partielle Veretherung umfasst und nachfolgend
(iii) nicht veretherte Dimethylbutene hydriert werden,
um eine tert.-Hexylmethyletherzusammensetzung zu bilden, die MDMB und Dimethylbutane umfasst.

18. Gemisch nach einem der vorhergehenden Ansprüche, bei dem Zusammensetzung (b) auch Dimethylbutene enthält.

19. Gemisch nach einem der vorhergehenden Ansprüche, bei dem Zusammensetzung (b) auch weniger als 1 % Methanol enthält.

20. Gemisch nach einem der vorhergehenden Ansprüche, bei dem Zusammensetzung (b) auch weniger als 5 % Olefine enthält.

21. Gemisch nach einem der vorhergehenden Ansprüche, bei dem Zusammensetzung (b) mehr als 50 Gew.%, vorzugsweise 60 Gew.% bis 100 Gew.% und insbesondere mehr als 80 Gew.% des tert.-Hexylmethylethers enthält.

22. Gemisch nach einem der vorhergehenden Ansprüche, das eine ausreichende Menge Zusammensetzung (b) enthält, um die Oktanzahl von Komponente (a) um mindestens 1 Einheit zu steigern, während gleichzeitig der Reid-Dampfdruck von Komponente (a) um weniger als 13,8 kPa (2 psi), vorzugsweise weniger als 6,9 kPa (1 psi) und insbesondere weniger als 3,4 kPa (0,5 psi) erhöht wird.

23. Verwendung einer tert.-Hexylmethyletherkomponente, die MDMB in einer Menge von mindestens 10 Gew.% umfasst, bezogen auf das Gesamtgewicht der tert.-Hexylmethyletherkomponente, und eine Misch-RON größer als 100 und eine Misch-MON größer als 90 hat, als Oktanzahlsteigerungsmittel für Motorbenzin.

24. Verwendung einer tert.-Hexylmethyletherkomponente, die MDMB in einer Menge von mindestens 10 Gew.% umfasst, bezogen auf das Gesamtgewicht der tert.-Hexylmethyletherkomponente, als Oktanzahlsteigerungsmittel für Motorbenzin, wobei die Misch-RON und/oder die Misch-MON der tert.-Hexylmethyletherkomponente höher als die RON und/oder MON des unbehandelten Motorbenzins ist.

25. Verwendung einer tert.-Hexylmethyletherkomponente gemäß Anspruch 23 oder 24, wobei der Reid-Dampfdruck des behandelten Motorbenzins um weniger als 13,8 kPa (2 psi), vorzugsweise weniger als 6,9 kPa (1 psi) und insbesondere weniger als 3,4 kPa (0,5 psi) höher ist.

## Revendications

1. Mélange comprenant
(a) de l'essence pour moteurs ou une matière première d'essence pour moteurs ; et
(b) une quantité, à effet d'augmentation d'indice d'octane, d'un constituant tertio-hexylméthyléther comprenant du 2-méthoxy-2,3-diméthylbutane (MDMB) en une quantité d'au moins 10 % en poids sur la base du poids total du tertio-hexylméthyléther,
dans lequel la composition (b) a un indice d'octane recherche (RON) et/ou un indice d'octane moteur (MON) supérieurs à ceux de la composition (a).

2. Mélange suivant la revendication 1, dans lequel la composition (b) a un RON supérieur à 95 et/ou un MON supérieur à 85.

3. Mélange suivant l'une quelconque des revendications précédentes, dans lequel la composition (b) a un RON supérieur à 105 et/ou un MON supérieur à 95.

4. Mélange suivant l'une quelconque des revendications précédentes, dans lequel le constituant tertio-hexylméthyléther de la composition (b) représente une proportion supérieure à 10 %.

5. Mélange suivant l'une quelconque des revendications précédentes, dans lequel le constituant tertio-hexylméthyléther de la composition (b) comprend 20 à 100 % en poids de MDMB.

6. Mélange suivant l'une quelconque des revendications précédentes, dans lequel le constituant tertio-hexylméthyléther de la composition (b) représente une proportion de 50 à 100 %.

7. Mélange suivant l'une quelconque des revendications précédentes, dans lequel le constituant tertio-hexylméthyléther de la composition (b) comprend plus de 80 % en poids de MDMB.

8. Mélange suivant l'une quelconque des revendications précédentes, dans lequel le constituant tertio-hexylméthyléther a un RON supérieur à 100 et/ou un MON supérieur à 90.

9. Mélange suivant l'une quelconque des revendications précédentes, dans lequel le constituant tertio-hexylméthyléther a un RON de mélange supérieur à 100 et/ou un MON de mélange supérieur à 90.

10. Mélange suivant l'une quelconque des revendications précédentes, dans lequel le constituant MDMB a un RON supérieur à 105 et/ou un MON supérieur à 95.

11. Mélange suivant l'une quelconque des revendications précédentes, dans lequel le constituant MDMB a un RON de mélange supérieur à 105 et/ou un MON de mélange supérieur à 95.

12. Mélange suivant l'une quelconque des revendications précédentes, qui a un RON supérieur à 90 et/ou un MON supérieur à 80.

13. Mélange suivant l'une quelconque des revendications précédentes, qui a un RON supérieur à 93 et/ou un MON supérieur à 83.

14. Mélange suivant l'une quelconque des revendications précédentes, qui contient une quantité suffisante de composition (b) pour augmenter l'indice d'octane du constituant (a) d'au moins 1, avantageusement d'au moins 2 et de préférence d'au moins 3 unités.

15. Mélange suivant l'une quelconque des revendications précédentes, qui comprend plus de 1 %, avantageusement plus de 2 % et de préférence plus de 5 % en volume de MDMB.

16. Mélange suivant l'une quelconque des revendications précédentes, dans lequel la composition (b) est préparée par un procédé comprenant les étapes consistant :
(i) à dimériser du propylène pour former des diméthylbutènes ; et
(ii) à éthérifier les diméthylbutènes avec du méthanol,
pour former la composition désirée.

17. Mélange suivant la revendication 16, dans lequel l'étape (ii) comprend une éthérification partielle et est suivie par
(iii) l'hydrogénation des diméthylbutènes non éthérifés
pour former une composition de tertio-hexylméthyléther comprenant du MDMB et des diméthylbutanes.

18. Mélange suivant l'une quelconque des revendications précédentes, dans lequel la composition (b) contient également des diméthylbutènes.

19. Mélange suivant l'une quelconque des revendications précédentes, dans lequel la composition (b) contient également moins de 1 % de méthanol.

20. Mélange suivant l'une quelconque des revendications précédentes, dans lequel la composition (b) contient également moins de 5 % d'oléfines.

21. Mélange suivant l'une quelconque des revendications précédentes, dans lequel la composition (b) contient plus de 50 %, avantageusement 60 % à 100 % et de préférence plus de 80 % en poids du tertio-hexylméthyléther.

22. Mélange suivant l'une quelconque des revendications précédentes, qui contient une quantité suffisante de composition (b) pour augmenter l'indice d'octane du constituant (a) d'au moins une unité, tout en augmentant en même temps la pression de vapeur Reid du constituant (a) de moins de 13,8 kPa (2 psi), avantageusement de moins de 6,9 kPa (1 psi) et de préférence de moins de 3,4 kPa (0,5 psi).

23. Utilisation d'un constituant tertio-hexylméthyléther comprenant du MDMB en une quantité d'au moins 10 % en poids sur la base du poids total du constituant tertio-hexylméthyléther et ayant un RON de mélange supérieur à 100 et un MON de mélange supérieur à 90, comme composant à haut indice d'octane pour une essence pour moteurs.

24. Utilisation d'un constituant tertio-hexylméthyléther comprenant du MDMB en une quantité d'au moins 10 % en poids sur la base du poids total du constituant tertio-hexylméthyléther, comme composant à haut indice d'octane pour une essence pour moteurs, dans laquelle le RON de mélange et/ou le MON de mélange du constituant tertiohexyl-méthyléther sont supérieurs au RON et/ou au MON de l'essence non traitée pour moteurs.

25. Utilisation d'un constituant tertio-hexylméthyléther suivant la revendication 23 ou 24, dans lequel la pression de vapeur Reid de l'essence traitée pour moteurs est supérieure de moins de 13,8 kPa (2 psi), avantageusement de moins de 6,9 kPa (1 psi) et de préférence de moins de 3,4 kPa (0,5 psi).
